

# UNITED STATES PATENT OFFICE.

HENRY HOWARD GREENWAY, OF CLARE, SOUTH AUSTRALIA, AND ALFRED HENRY PIPER LOWRY, OF PRAHRAN, VICTORIA, AUSTRALIA.

## ORE CONCENTRATION.

1,102,738.

Specification of Letters Patent.

Patented July 7, 1914.

No Drawing.

Application filed May 17, 1913. Serial No. 768,374.

To all whom it may concern:

Be it known that we, HENRY HOWARD GREENWAY, analytical chemist and metallurgist, of Clare, State of South Australia, 5 Commonwealth of Australia, at present of 34 Queen street, Melbourne, State of Victoria, Commonwealth of Australia, and ALFRED HENRY PIPER LOWRY, metallurgist, of "Lynzala," High street, Prahran, State of 10 Victoria aforesaid, have invented certain new and useful Improvements in Ore Concentration, of which the following is a specification.

This invention relates to improvements in 15 ore concentration and has for its object the separation of various metallic sulfids from each other by means of flotation separation.

In this specification the word "ores" is intended to include concentrates, tailings 20 slimes or other products containing mixed metallic sulfids.

We have discovered that if a salt of chromium (such as sodium bichromate or potassium bichromate) is introduced in solution 25 into the circuit liquors, or if the material to be treated is subjected to the action of such chromium salt solution by digestion or otherwise that the sulfids are affected in such a way as to leave certain of them amenable to flotation separation while certain other of them are rendered relatively not 30 amenable to flotation whereby products are obtained relatively high in certain sulfids on the one hand and relatively high in other sulfids on the other hand.

According to this invention the mixed sulfid ores after pulverization are introduced into water containing in solution, a salt of chromium (such as sodium or potassium 40 bichromate) and also a small percentage of an air emulsifying agent for example an essential oil (say eucalyptus) and the mixture is thoroughly agitated and submitted to a flotation separation, the result of which is 45 to cause certain of the sulfids to float in the form of a froth or scum which can be separated by any well known means, leaving in the residue the other sulfids which are not susceptible to flotation.

50 In some instances it may be advisable to digest the pulverized mixed sulfid ores in water containing in solution a salt of chromium (such as sodium bichromate or potassium bichromate) and after removing the 55 surplus solution subsequently submitting the

said mixed sulfid ores to a flotation separation.

If desired the resulting products may be retreated by the same process with or without the addition of fresh quantities of the 60 substances referred to.

The following are examples of the application of this invention:

(1.) A molybdenum ore containing 15% molybdenite and 25% iron pyrites was 65 crushed to pass 100 mesh, and then subjected to froth flotation treatment in apparatus of well known type by being first of all vigorously agitated with four times its weight of water at 120° F. containing in 70 solution 0.25% of sodium bichromate to which was added eucalyptus oil in the proportion of one pound per ton of ore treated. The flotation product obtained from this operation consisted of a concentrate containing 75 93% molybdenite and 4.9% iron pyrites.

(2.) A copper ore containing 6.5% copper and 35% iron was crushed to pass 100 mesh. This was digested in a hot solution containing 80 1% sodium bichromate for a period of about 30 minutes. The digestion liquor was then decanted and the material was subjected to froth flotation separation using water only to which was added a frothing agent (viz, eucalyptus oil) in the proportion of 1 pound per ton of material treated, producing a flotation product containing 1.9% copper and 30.2% iron, leaving a residue containing 0.7% copper and 36.2% iron. 85

(3.) A lead-zinc slime containing 18.6% lead and 32.2% zinc was digested for thirty minutes in warm water containing in solution 1% of sodium bichromate. The solution was decanted and the material subjected to the froth flotation separation using water only to which was added eucalyptus oil in the proportion of 1 lb. per ton of slime treated producing a flotation product containing 47.2% zinc and 6.3% lead, leaving a residue containing 31.6% lead and 16.3% zinc. 95 100

In most instances the action is facilitated by heating the solutions, and we have found temperatures of from 120° F. to 150° F. to 105 be in most cases suitable.

We do not confine ourselves to the proportions above given: the best proportion in each case can be determined by trial.

Having now fully described and ascer- 110

tained our said invention and the manner in which it is to be performed we declare that what we claim is:—

1. A process of concentrating metalliferous ores, which consists in subjecting the ore to the action of a chromium salt and to flotation separation whereby products are obtained relatively high in certain values and other products are obtained relatively high in other values.
2. A process of concentrating metalliferous ores, which consists in subjecting the ore to the action of a chromium salt and to agitation with a frothing agent to produce a froth relatively high in certain values of the ore.
3. A process of concentrating metalliferous ores, which consists in subjecting the ore to digestion in a solution of a chromium salt, and then to flotation separation, whereby products are obtained relatively high in certain values and other products are obtained relatively high in other values.
4. A process of concentrating metalliferous ores, which consists in subjecting the ore to digestion in a solution of a chromium salt, and then to agitation with a frothing agent to produce a froth relatively high in certain values of the ore.
5. A process of concentrating ores, which consists in subjecting an ore containing zinc and lead sulfids to the action of a chromium salt and to a flotation separation, whereby there is produced a flotation product relatively high in zinc and low in lead and a

residue relatively high in lead and low in zinc.

6. A process of concentrating ores, which consists in subjecting an ore containing zinc and lead sulfids to the action of a chromium salt and to agitation with a frothing agent to produce a froth relatively high in zinc and low in lead leaving a residue relatively high in lead and low in zinc.

7. A process of concentrating ores, which consists in subjecting an ore containing zinc and lead sulfids to digestion in a solution of a salt of chromium, and then to flotation separation, whereby a float concentrate is obtained relatively high in zinc and low in lead and a residue is obtained relatively low in zinc and high in lead.

8. A process of concentrating ores, which consists in subjecting an ore containing zinc and lead sulfids to digestion in a solution of a salt of chromium, and then to agitation with a frothing agent to produce a froth relatively high in zinc and low in lead, leaving a residue relatively low in zinc and high in lead.

In testimony whereof we, the said HENRY HOWARD GREENWAY and ALFRED HENRY PIPER LOWRY, have signed our names to this specification in the presence of two subscribing witnesses.

HENRY HOWARD GREENWAY.  
ALFRED HENRY PIPER LOWRY.

Witnesses:

CHARLES NICHOLAS COLLISON,  
DAISY WILLIAMS.